

Sept. 5, 1933.

S. P. MILLER

1,925,150

PITCH COMPOSITION AND METHOD OF MAKING SAME

Filed Aug. 17, 1927

2 Sheets-Sheet 1



INVENTOR  
*Stuart Parmalee Miller*  
BY  
*Pennie Davis, Marvin & Edwards*  
ATTORNEYS

Sept. 5, 1933.

S. P. MILLER

1,925,150

PITCH COMPOSITION AND METHOD OF MAKING SAME

Filed Aug. 17, 1927

2 Sheets-Sheet 2



Fig. 2.

INVENTOR  
*Stuart Parmelee Miller*  
BY  
*Perrie Davis, Merritt & Edwards*  
ATTORNEYS

## UNITED STATES PATENT OFFICE

1,925,150

PITCH COMPOSITION AND METHOD OF  
MAKING SAME

Stuart Parmelee Miller, Glen Ridge, N. J., assignor to The Barrett Company, New York, N. Y., a corporation of New Jersey

Application August 17, 1927. Serial No. 213,497

2 Claims. (Cl. 202—30)

This invention relates to a new pitch composition and to an improved method for producing the same. The invention also includes improvements in distillation of tar, and in the recovery and production of valuable products therefrom.

In order to produce heavy or high boiling point oils from tar by ordinary distillation methods, it is necessary to carry the distillation to a high temperature. Such distillation is accompanied 10 with a very considerable decomposition of oil constituents of the tar, so that the yield of oils recovered by distillation is considerably less than that contained in the tar distilled, while an increased amount of pitch is produced, partly by 15 decomposition during the distillation, and the pitch has a high carbon content.

Such distillation of tar is commonly carried out at tar distillation plants located at a greater or less distance away from the coke oven plant at 20 which the tar is produced. The tar separated from the coke oven gases by cooling and condensation is collected and transported to the tar distillation plant and there subjected to distillation. Such procedure is accompanied by cost of 25 transportation and losses of tar incidental to its handling and shipment, while the distillation of the tar is accompanied with further loss of oil by decomposition and increase in the amount of pitch and carbon content of the pitch produced 30 as a residue of the distillation. When such high carbon pitch is blended with ordinary tar, the high carbon content of the pitch may interfere materially with the blending operation and may result in settling out of some of the carbon with 35 resulting lack of homogeneity of the blended product and with liability of clogging of pipe lines, etc., where the resulting blended product is used for fuel or other purposes.

The present invention eliminates the necessity 40 of the transportation of tar from a coke oven plant to a tar distillation plant, with its attendant expense and incidental loss in handling and transportation, and provides an improved process, whereby heavy oils and a blended pitch composition of improved properties are directly produced at a coal distillation plant, such as a coke oven plant.

According to the present invention, the tar, such as is produced from coke oven gases in ordinary coke oven by-product operation, is subjected 50 to distillation by bringing it directly into contact with the hot coal distillation gases at the coke oven plant, and distillation is so carried out as to produce a hard or high melting point pitch, which 55 will, nevertheless, have a much lower carbon con-

tent than the pitch produced by ordinary tar distillation methods in externally heated tar stills; and this pitch directly produced by such distillation is then blended with tar to form a composite product valuable, for example, for use 60 as a fuel composition in open hearth furnaces, etc. The production of the pitch in this way is accompanied by the production of a high yield of oils, including heavy or high boiling point oils, and including oils which, in ordinary tar distilla- 65 tion methods, are decomposed and converted into a pitch residue or into carbon or other decomposition products.

The gases from coke ovens or retorts leave the ovens at a high temperature, around 600° to 700° C. or higher, and are commonly cooled in the collector main of the battery by the introduction of ammonia liquor or ammonia liquor and tar, directly into the collector main to throw down a heavy tar from the gases, and by further cooling 75 of the gases in the coolers or condensers to throw down a light tar or tarry oil therefrom. The heavy tar and light tar are commonly mixed and subjected to distillation. The tar so produced may be employed in the process of the present 80 invention, and may be tar produced at the same coke oven plant at which the distillation is carried out or it may be coke oven tar produced at another coke oven plant, or may be in part gas house tar or water gas tar, etc. 85

According to the present invention, the tar is subjected to distillation by bringing it into direct contact with the hot coke oven gases at a sufficiently high temperature to distill the tar to remove a large part of the oil components thereof, 90 and to leave a pitch residue of high melting point but of relatively low carbon content; and the resulting pitch is then blended with raw tar or with heavy tar, etc., to form the new pitch composition. The distillation of the tar in direct 95 contact with the hot coke oven gases can be carried out, for example, in accordance with the processes described in my prior applications, Serial Nos. 166,081, 171,955, 172,962, and 181,366, by spraying the tar into the hot coke oven gases at 100 a temperature not greatly below that at which the gases leave the ovens, so as to use the high temperature of the gases for the distillation. Such distillation will take place without external heating of the apparatus in which the distilla- 105 tion takes place, and with heating of the tar only by the hot coal distillation gases. This distillation will remove from the individual particles of tar sprayed into the gases a large part of the vaporizable components, leaving a pitch residue 110

which will vary in its melting point with the extent to which the distillation is carried. Such distillation of the tar by direct contact with the gases avoids the local over-heating which takes place in externally heated tar stills, and, where the tar is not kept in contact with the hot gases for a prolonged period, can be carried out without any considerable increase in carbon content due to decomposition during the distillation, although some such decomposition may take place, particularly where the time of contact of the tar and resulting pitch residue with the hot gases is prolonged. In any event, the pitch residue produced will be of relatively much lower carbon content than pitch residues produced by distillation in ordinary externally heated tar stills, while a considerably increased oil yield can be obtained by distillation from the same amount of tar, as compared with the oil yield produced by distillation in ordinary tar stills.

The present invention, accordingly, forms a valuable process for the distillation of tar where a part only of the tar is to be distilled, and where the maximum oil yield is desired from the tar and where the pitch residue is to be employed for blending with the remainder of the tar for fuel or other purposes.

The distillation of the tar and the production of the pitch, according to the present invention, are advantageously carried out as a continuous operation, with the continuous production of a hard, high melting point pitch, and with the continuous blending of such pitch with raw tar to produce the new composite pitch composition. The tar can be introduced, for example, directly into a still through which the hot coke oven gases are passing and the rate of distillation regulated or the tar recirculated and further distilled, to give continuously a high melting point pitch; and this pitch as produced can then be advantageously blended continuously with a stream of raw tar to form continuously the blended composite pitch products.

The hot coke oven gases coming from the individual coke ovens at a high temperature are capable of distilling an amount of tar many times that which is produced from the gases from a single oven. Accordingly, in a coke oven plant where the tar to be distilled is that produced at the same plant, the gases from a few only of the ovens will suffice for the distillation of the tar produced from the remainder of the battery. Where, however, the tar from several batteries is to be distilled, the gases from an increased number of ovens, or from an entire battery, or from so much of a battery as is connected to a single collector main, may be employed for the distillation. By bringing the tar intimately into contact with the hot gases at substantially their maximum temperature as they leave the coke oven, the tar can be continuously distilled in a single operation to produce substantially the maximum yield of distillate and a hard high melting point pitch residue, which can be drawn off continuously and blended continuously with raw tar, etc., to form the new pitch composition. In order to obtain substantially the maximum yield of distillate, the distillation can be carried to such an extent that pitch of high melting point, for example, pitch of 300° F. melting point, can be produced; but the further distillation can advantageously be carried to such an extent that a much higher melting point pitch is produced, such as a pitch of melting point around 400° F., or in some cases as high as 500° F. The distil-

lation of tar to produce such a high melting point pitch gives a heavy distillate which contains constituents normally semi-solid or solid and grease-like or resinous in character, in an isolated state, but which, when condensed with lighter oils, blend therewith to form a homogeneous product.

The blending or mixing of the pitch with the tar can be carried out as successive batches by adding the hot pitch gradually to a tank of hot tar, or vice versa. It can also advantageously be carried out in a continuous manner by running streams of pitch and tar continuously into a mixing box or receptacle in which the streams blend and mix with each other to form a homogeneous product, with further agitation, if necessary, and by continuously discharging the resulting homogeneous mixture from the mixing chamber. When tar is distilled to produce pitch of high melting point, and where the pitch is directly blended with raw tar, the hot pitch will heat the tar and result in a heated mixture from which more or less distillation may take place, due to the heating of the tar to a temperature above the distillation temperature of some of its constituents. The oils so distilled from the tar may be removed and recovered as a distillate oil, or may be refluxed back and blended with the pitch composition. Raw tar which contains water will be dehydrated by the mixing operation, but by running streams of the raw tar and hot pitch into a mixing box, any foaming due to the removal of water will be taken care of without interfering with the mixing operation.

The resulting blended product made by blending the hot pitch and tar can be employed for various purposes, such as for fuel purposes, as fuel in open hearth furnaces, etc.; or it can be employed for other purposes where a blended pitch and tar product is desired, for example, for road-making purposes, or for roofing, etc.

The tar which is blended with the hot pitch may be part of the tar produced at the same coke oven plant, or it may be tar from another plant, or gashouse tar, etc. Instead of using the total tar, including both the heavy tar from the collector main and the light tar or tarry oil from the condenser, only the heavy tar from the collector main may be blended with the hot pitch, leaving the tarry oil from the condensers to be employed for other purposes. Such tarry oil can advantageously be blended with the distillate condensed from the enriched gases resulting from the distillation of the tar and production of the pitch, and a blended product may thus be obtained which can be employed directly for creosoting or other purposes. The present invention includes the production of such a blended product from the distillate and from light tarry oils as well as the production of a composite pitch product from the pitch residue of the distillation and the heavy tar from the collector main.

The distillation of the tar by the hot coke oven gases will result in a very material enrichment of the gases in oil vapors, and the oil condensed from the resulting enriched gases will contain a relatively low content of heavy tarry matter, since they will be made up largely of the distillate oils and will contain a relatively small amount of oils and heavy tar directly condensed from the gases employed for the distillation and originally carried thereby before the enrichment by the distillation. The enriched gases can be employed with whatever heavy tar or pitch constituents they contain and blended,

80

85

90

95

100

105

110

115

120

125

130

135

140

145

150

for example, with the light tar or tarry oils directly produced from coke oven gases in the ordinary condensers or coolers of the by-product recovery system. In such case, only the 5 heavy tar from the collector mains may be subjected to distillation for the production of the pitch residue, and the light tar or tarry oils from the condensers may be kept separate and blended with the distillate from the distillation 10 of the heavy tar in such proportions as will give, for example, a creosote composition suitable for use as a substitute for ordinary coal tar solution. Such a creosote composition is described in my prior application, Serial No. 199,629.

15 The gases produced by the distillation can be subjected to a cleaning treatment at a high temperature with an electrical precipitator to remove suspended pitch particles therefrom, and to leave only gases carrying only clean oil vapors, 20 from which clean oils free from tar can then be directly condensed. In this case an added amount of pitch will be recovered from the electrical precipitator, which may be blended with the pitch resulting from the distillation. In this 25 case only pitch and clean oils will result from the distillation, and the clean oils may be recovered as merchantable oils, for example, clean creosote oils, or as a creosote oil fraction and a tar acid oil fraction, as described, for example, 30 in my companion applications Serial Nos. 206,366 and 206,367.

The new pitch composition of the present invention differs greatly from compositions made by mixing tar with pitch produced by distilling 35 tar in simple, externally heated tar stills. In such stills of, for example, 10,000 gallons capacity, where successive charges of tar are heated and distilled by the application of external heat to the still, the yield of distillate oil is relatively. 40 small, and the amount of pitch produced is large and the pitch is high in free carbon, and particularly in carbon produced by decomposition during the distillation. Tar distilled in such stills to produce a pitch of melting point around 170° 45 F. gives an oil yield of only about 33 per cent of the tar distilled; if the distillation is carried further to produce a pitch of around 200° F. melting point, the oil yield is only about 38 per cent, while if the distillation is carried still further to 50 produce a pitch of around 300° F. melting point, the oil yield is increased only to about 44 per cent, and coking of the tar may begin before pitch of a melting point of around 400° F. is reached. The distillation of tar with hot coke 55 oven gases, as carried out in producing the new pitch composition, gives a radically increased yield of oils and a corresponding reduction in the amount of pitch and an entirely different character of pitch. For example, in distilling 60 certain coke oven tars by direct contact with hot coke oven gases where the time of contact is short, the distillation of the tar to produce a pitch of a melting point around 170° F. gives an oil yield around 48 per cent; while with 65 distillation to produce a pitch residue of melting point around 200° F., an oil yield around 55 per cent or higher can be obtained; and if the distillation is carried so far as to produce pitch of a melting point around 300° F., an oil yield around 70 per cent can be obtained; and it is possible to carry the distillation to produce pitch of 400° F. melting point and higher, with a yield, for example, around 80 percent of oil when 400° F. melting point pitch is produced. Comparing, 75 for example, the pitches of melting point around

300° F. produced respectively in ordinary externally heated tar stills of the type above mentioned, and pitch of similar melting point produced by direct distillation with hot coke oven gases, it will be seen that the yield of oils is only 80 about 44 per cent in one case and around 70 per cent in the other. The remaining 26 per cent of oil is largely decomposed by the distillation in the ordinary tar stills, with increase in pitch residue. Moreover, this decomposition, due to 85 local overheating, etc., results in production of a large amount of carbon, and of carbon of a different character. It includes not only substances commonly called "carbon" because insoluble in benzol, but it contains considerable elemental carbon or decomposition products insoluble, for example, in anilin, while the so-called carbon contained in the pitch employed in the new composition is readily soluble in anilin and is composed of heavy hydro-carbons, which are readily soluble in, or form a homogeneous composition with, the tar with which the pitch is blended. The avoidance of the large increase in carbon of a different character in the pitch products employed in the new composition gives an 100 improved composition from which there is little, if any, liability of carbon settling out, for example, in pipe lines by which the composition is supplied to fuel burners.

The invention will be further described in connection with the accompanying drawings, which illustrate in a somewhat conventional and diagrammatic manner an arrangement of apparatus suitable for the practice of the invention.

In the accompanying drawings, 110 Fig. 1 shows an arrangement of part of a coke oven plant with part of the by-product recovery system, including an arrangement for distilling tar by direct contact with hot coke oven gases; and

Fig. 2 is an elevation with parts in section of the short collector main and electrical precipitator of Fig. 1.

In the accompanying drawings, the coke oven 1 has the usual uptake pipes 2 leading to the ordinary collector main 3, having center box 4 and cross-over main 5 for leading the gases to the condensers shown as 6 and 7, which are of the direct type cooled by introduction of cooling liquid, such as water or ammonia liquor, through the pipes 8. From condensers the gases pass to the exhauster 9, and then to the ammonia absorber and light oil scrubber (not shown). 125

Ammonia liquor, or ammonia liquor and tar, is commonly supplied to the collector main to cool the gases therein and to separate tar therefrom and to flush the tar from the collector main through the center box. The outlet for tar and liquor is indicated at 10 and leads to the separator or decanter 11, from which the tar flows to the tar storage or receiving tank 12, and the ammonia liquor to the tank 13. The line 15, with pump 14 in it, conveys tar to a short collector main 21 for distillation. 130

The tarry oils condensed in the condensers 6 and 7 are run off through lines 16 and 17 and may be collected together in the receiver or decanter 18, from which the ammonia liquor is collected in the receiver 20, and the tarry oils in the receiver 19. 140

The tar from the receiver 12, or tar from another source supplied through the line 41, is introduced into the short collector main 21, which is arranged at the back of the coke oven battery and connected with a limited number of uptake pipes 150

22, so that the gases from as many ovens as may be required for distillation can be supplied to the short collector main for such distillation. The tar is introduced into the short collector main 5 through spray nozzles 23, and is brought into intimate contact with the hot gases passing through the short collector main, and is thereby distilled and a pitch residue produced. A pump 14' is provided through which the pitch residue may be 10 recirculated. The hot gases coming from the individual ovens are at a high temperature, around 600° to 700° C. or higher, and with insulation of the individual uptake pipes and of the short collector main, these gases enter the short 15 collector main without any considerable reduction in temperature, so that they are available at a high temperature for distillation of the tar. By regulating the tar supply, and by recirculating the resulting pitch if necessary, the tar can be distilled to produce a pitch of high melting point, from which a high yield of oils is driven off.

The pitch residue from the distillation goes through the line 24 to a mixing tank or chamber 25, to which tar is also supplied in regulated 25 amounts through the line 26. With continuous distillation of tar and continuous production of pitch, the pitch can be supplied continuously to the mixing chamber, together with continuous supply of tar in regulated amount so that the 30 pitch and tar will continually mix in the mixing chamber and the mixture will flow out through the outlet 30 to the receptacle 31 for the mixed product.

The hot pitch will enter the mixing chamber 25 at a high temperature, while crude tar, or even wet tar, may enter through the line 26 at ordinary temperature. The heat of the hot pitch will serve to heat the tar with which the pitch admixes, and this in turn will serve to dehydrate 40 the tar and remove therefrom more or less of the oils volatile at the temperature of the resulting mixture. Some foaming may take place where the hot pitch and the wet tar come into contact with each other, but this will be unobjectionable, 45 because the mixing chamber 25 can be kept nearly empty, that is, with only a layer of the flowing mixture in the bottom, so that any foam formed will be taken care of. The mixing chamber 25 may be supplied with an agitator to promote the 50 intermixture of the tar and pitch, but ordinarily this will not be necessary where regulated streams of the two materials are suitably brought together in the mixing chamber. The hot pitch, because of its low carbon content, and because the 55 carbon content which it contains is largely made up of heavy hydrocarbons, readily blends with the tar to form a substantially homogeneous mixture with little, if any, tendency for the separation of carbon therefrom during storage and circulation 60 to burners, etc.

Oils vaporized in the mixing chamber can be condensed by the condenser 27 and either returned to the mixture of tar and pitch through the line 28, or drawn off as condensate through 65 the line 29 and employed as an oil for other purposes.

The gases leaving the short collector main will be materially enriched in vapors due to the distillation. These gases pass through the line 32 70 to the condensing system shown in two condensers 34 and 35. The gases may be passed to this condenser without further treatment by cleaning, but are advantageously subjected to cleaning with an electrical precipitator at a high temperature 75 to recover suspended pitch particles therefrom

in the form of a pitch product which can advantageously be added as part of the new fuel composition. The gases from the short collector main will leave it while still at a high temperature, and if passed through the electrical precipitator without material cooling, will carry pitch particles of relatively a high melting point pitch and will carry a large amount of oils in the form of vapors. By treating the gases and separating the suspended pitch particles therefrom, the pitch can be employed in making the new pitch composition while the gases can be subjected to cooling and condensation to recover directly therefrom clean oils, free or substantially free from heavy tar and pitch impurities. These clean oils will be condensed in the condensers 34 and 35 which may be of the indirect type, i. e., cooled by indirect contact with water, so that a heavy creosote oil and a lighter tar acid oil can be directly recovered therefrom. The gases then pass to the exhauster 36 and to an ammonia absorber, etc., (not shown).

The clean oils recovered in the condensers 34 and 35 may be blended with the tarry oils recovered in the main condensing system in proper proportions to give a creosoting composition; or only the heavy condensate from the condenser 34 may be so employed. If the gases are not cleaned with an electrical precipitator, they will carry more or less heavy tar and pitch constituents with them, and the oils condensed in the condensers 34 and 35 will be tarry oils. They will differ materially, however, from the tarry oils collected in the receiver 19, because they will be recovered or condensed from enriched gases, and will contain relatively little pitch and heavy tar constituents. The tarry oils from the respective systems can advantageously be blended in proper proportions to give directly a creosoting composition suitable for use as an improved sub- 110

stituents with them, and the oils condensed in the condensers 34 and 35 will be tarry oils. They will differ materially, however, from the tarry oils collected in the receiver 19, because they will be recovered or condensed from enriched gases, and will contain relatively little pitch and heavy tar constituents. The tarry oils from the respective systems can advantageously be blended in proper proportions to give directly a creosoting composition suitable for use as an improved sub- 115

The apparatus illustrated includes the by-product recovery system of an ordinary coke oven plant in which ammonia liquor is employed for cooling the gases in the collector main, and in 120 which a heavy tar is separated from the collector main and tarry oils from the condensers. In addition, the apparatus illustrated includes a tar still for distilling the tar by direct contact with hot coke oven gases from part of the battery so 125 as to produce from this tar a pitch residue and distillate oils which may be clean distillate oils, or which may be tarry oils. The pitch residue is then blended with tar to form the new fuel composition. The oils resulting from the distillation may likewise be blended with the tarry oils from the ordinary recovery system to make 130 a creosoting composition, while only the heavier tar from the collector main of the ordinary system may be subjected to distillation to produce 135 a pitch residue and distillate oils therefrom.

The present invention involves the production of a new fuel composition, in which the pitch directly produced by distillation of tar with hot coal distillation gases and of the distinctive composition resulting from such distillation is blended with tar or heavy tar or tar from another source such as gashouse tar, or water gas tar, to make a new composite product suitable for use, for example, for fuel and other purposes. The process includes the production of a high yield of oils, such as creosote oils, with a relatively low yield of pitch from the tar distilled, but with advantageous employment of this pitch by blending it with undistilled tar, or with heavy tar, etc. 150

in a manner which makes the pitch available to advantage for fuel and other purposes. The composite pitch product can be employed, for example, for roofing purposes, or for road treating purposes, etc. Simultaneously with the production of the new pitch composition, there may advantageously be also produced a creosoting composition by blending the distillate oils resulting from the distillation with directly recovered tarry oils in suitable proportion.

In this way the total tar produced by the coke oven plant may be used up and converted into the new fuel composition and into compositions suitable for use directly for creosoting purposes.

When the tarry oils, as well as the heavy tar from the ordinary by-product system, are subjected to distillation to produce the pitch for blending to make the new product and to produce distillate oils, the distillate oils can be employed as such or blended with other products. Instead of working up all of the tar from the coke oven battery by distillation, part of it may be employed for blending with the pitch produced by the distillation, or the pitch so blended may be tar from another source, and even tar of different properties, such as, for example, water gas tar. Fuel compositions made from the high melting point low carbon pitch and water gas tar are advantageous, inasmuch as water gas tar itself is not suitable for distillation to give distillate oils suitable for certain purposes, such as creosoting purposes, or it gives distillate inferior for that purpose. By subjecting coal tar to distillation to recover creosote oils, and then blending the pitch residue with water gas tar, a valuable fuel composition is obtained.

I claim:—

1. The method of producing pitch compositions and creosoting compositions, which comprises cooling hot untreated coke oven gases to separate therefrom first a heavy tar and thereafter a light tar, subjecting the heavy tar to distillation by bringing it into direct contact with hot coke oven gases, at substantially the temperature at which they leave the ovens to produce a pitch residue of high melting point and gases enriched in oil vapors, mixing the resulting hot pitch residue with tar to form a homogeneous pitch composition, cooling the enriched gases to condense oil vapors therefrom and mixing the oil condensed from the gases with the light tar to form a composition suitable for use for creosoting purposes.

2. The method of producing composite pitch compositions and clean oils, which comprises subjecting tar from gasification or coal carbonization processes to distillation by bringing it into direct contact with hot coke oven gases to produce a pitch residue of at least 300° F. melting point and gases enriched in oils, subjecting the resulting gases to cleaning with an electrical precipitator to separate suspended pitch particles therefrom, combining the pitch from the precipitator and the pitch residue from the distillation while still hot and without substantially increasing the free carbon content of either with tar to form a composite pitch composition, and recovering clean oils from the gases resulting from the distillation.

STUART PARMELEE MILLER.

40

110

45

115

50

120

55

125

60

130

65

135

70

140

75

145

150